

## UNITED STATES PATENT OFFICE

1,939,659

## GUM INHIBITOR FOR HYDROCARBONS

William S. Calcott, Penns Grove, N. J., and Herbert W. Walker, Wilmington, Del., assignors to E. I. du Pont de Nemours & Company, Wilmington, Del., a corporation of Delaware

No Drawing. Application September 28, 1929  
Serial No. 395,988

10 Claims. (Cl. 44—9)

This invention relates to improvement in means for the protection of liquid hydrocarbon products against discoloration and formation of insoluble and gummy products, and more particularly to 5 improved materials for use with unsaturated liquid hydrocarbons which may be used as fuels.

Liquid hydrocarbons as commercially produced, particularly when prepared by the distillation or cracking of petroleum, possess a tendency to dis- 10 color on standing and to form gums and resinous substances. Gasolines produced by the modern cracking processes are extremely complicated mixtures comprising many constituents, the character of these constituents and the relative pro- 15 portions of different constituents depending upon the source of the crude and the particular cracking process employed. Besides the normal and branched chain paraffines, there are often present substantial percentages of aromatic hydrocarbons. 20 The crude cracked gasoline also always contains unsaturated hydrocarbons, such for example as olefines and diolefines. Although there may be present some compounds containing a triple bond, these are probably not compounds such as may be 25 formed by the polymerization of acetylene, but rather such compounds as may be formed by the isomerization of dienes and having the general formula  $C_nH_m$  where  $m$  is greater than  $n$ , but less than  $2n+2$ . These unsaturated compounds 30 in the presence of air are capable of oxidation to form a series of products, some of which are resinous or gummy. The diolefines, and more un- 35 saturated hydrocarbons, are particularly easily oxidized. Differences in structure other than the degree of unsaturation cause considerable variation in the tendency to oxidize, but in general the ease of oxidation increases with the degree of unsaturation. The more recent pressure methods 40 of vapor phase cracking result in a considerably higher percentage of diolefines than the older methods, and it has been stated that these products may run as high as 8 to 15% in unrefined gasoline.

It has been necessary to treat the crude products resulting from the more recent cracking processes in some manner to remove the greater part of these more highly unsaturated products. Among these methods of treatment may be mentioned the sulfuric acid treatment and the fuller's 50 earth vapor phase treatment. While these methods of purification may remove the greater part of the highly unsaturated compounds, it is found that many brands of gasoline tend to discolor on storage and to form a certain amount of gum. 55 The gum appears to be a complex mixture of

polymerized hydrocarbons, resins, acids, aldehydes, ketones and peroxides. Its formation is distinctly detrimental in all cases. For example, the deposition of gum in gasoline gives a sticky substance which deposits upon the walls and bottom of the container, and which may cause serious trouble if formed or deposited in the fuel system of internal combustion engines. The soluble portion of the gum is also objectionable because of the introduction of a non-volatile component into 60 the gasoline. 65

Our invention has for an object the inhibition of the formation of these insoluble gums and resins, with an attendant improvement in the quality of the hydrocarbon and freedom from the 70 difficulties introduced by the formation of the more or less insoluble and sticky, gummy material, such as irregular flow in the fuel and lubricating systems of internal combustion engines. A further object is to make it possible to 75 use as an internal combustion fuel, liquid hydrocarbons such as gasoline, that contain larger amounts of highly unsaturated compounds than commercially used at present. A product of this sort can be produced at a lower cost, and possesses 80 in certain cases, improved anti-knock properties.

We have found that by treating hydrocarbons, and specifically unsaturated hydrocarbons such as hydrocarbon fuels, and more specifically such as cracked gasoline or gasoline which has a 85 tendency to form gum, the gum formation can be very appreciably inhibited if the hydrocarbon is treated with a diaryl guanidine salt of a fatty acid. More specifically, our invention relates to the use as gum inhibitors for hydrocarbons of 90 compounds of the type



in which A is a fatty acid and in which R is an aryl group, and R' is an aryl group which may be the same as or different from R, and in which both R and R' may contain alkyl substituents. By way of illustrating our invention, we may set 100 forth the following examples:

Example 1

Diorthotolylguanidine-stearate was dissolved to the extent of 0.002% in an unstable gasoline 105 which, when untreated, developed considerable yellow color within from six to eight hours, and after three weeks time contained a large amount of insoluble gum and resin when placed in a glass bottle and exposed to sunlight. The identical 110

